

March 7, 1939.

H. RODMAN

2,149,747

CARBURIZER

Filed May 1, 1936

Fig. 3.



Fig. 1.



Fig. 2.



WITNESSES

A. B. Wallace,  
J. B. Flick.

INVENTOR

By Hugh Rodman  
Brown, Critchlow & Flick  
his ATTORNEYS.

## UNITED STATES PATENT OFFICE

2,149,747

## CARBURIZER

Hugh Rodman, Verona, Pa., assignor to Rodman Chemical Company, Verona, Pa., a corporation of Pennsylvania

Application May 1, 1936, Serial No. 77,329

6 Claims. (Cl. 148-30)

This invention relates to carburizing by the dry pack method.

It is among the objects of the invention to provide carburizing compounds which are of simple composition, possess satisfactorily high carburizing efficiency, are cheap, may be made by standard procedures and in any of the commercially desirable physical forms, and which minimize disadvantageous characteristics of many prior art carburizing compounds.

A further object is to provide carburizing compounds which exhibit carburizing activity at the usual carburizing temperatures and which in addition possess unusually well-sustained activity in repeated use and require therefore the addition of minimal amounts of fresh material.

Yet another object is to provide carburizing compounds embodying the foregoing advantageous characteristics and which not only are simpler in composition and cheaper than the carburizing compounds used commercially, but also are of at least equal, or comparable, carburizing efficiency.

Still another object is to provide carburizing compounds in which high and commercially acceptable carburizing activity is attained predominantly or exclusively by the use of lime and certain metal oxides referred to hereinafter, and in which the use of barium carbonate and other relatively expensive energizers, or of a plurality of energizers, is unnecessary.

Further objects are to provide carburizing compounds embodying the foregoing desirable features and characterized by other advantageous features, singly or in combination, such as production of smooth and evenly carburized surfaces, elimination of offensive and poisonous dust, and in the use of which attack upon the carburizing containers is repressed or eliminated.

The invention will be described in connection with the accompanying drawing, in which Fig. 1 is a graph showing the relative energizing powers of the commonly used alkali and alkaline-earth metal energizers as a function of their molecular weights; Fig. 2 a graph showing how the carburizing activity due to various energizers varies with the amount of energizer used in a carburizing compound; and Fig. 3 a graph illustrative of the present invention.

Carbon itself, at least in any of its common forms, possesses very low carburizing ability, and consequently the so-called energizers are mixed with carbon to provide a mixture which will cause carburization at a commercially acceptable rate.

The energizers commonly used, i. e., carbon-

ates or oxides of barium, sodium, and calcium, are not equally effective in increasing the carburizing power of carbon.

Lime, whether in the form of calcium carbonate or calcium oxide, has been considered to be a very inefficient energizer. In fact, used alone it possesses much less energizing power than either barium carbonate or sodium carbonate and as far as I am aware, it has not been possible heretofore to make a carburizing compound which will satisfy modern requirements by the use of lime as the sole energizer. It is ordinarily used in minor amount in carburizers, however, not to materially add to the energizing effect produced by barium carbonate, or other powerful energizer, but rather to minimize roughening of the surface of the steel which may be caused by the use of barium or sodium energizers alone.

These relations are represented in Fig. 1, which represents the relative energizing abilities of the individual energizers as determined from carburizing tests made of mixtures of 90 parts of a low-ash carbon and 10 parts of carbonate of the energizer (see, Trans. Amer. Soc. Steel Treatment, May 1925, p. 635). This shows that of the alkaline earths barium oxide has the greatest energizing power, while lime alone is indeed a very poor energizer so that it would be expected that lime would be incapable of highly energizing carbon.

As appears from Fig. 2, the effectiveness of an energizer increases with increase in the amount used until a maximum energizing effect is reached. But these curves show also that even with as much as 30 per cent of lime, the carburizing activity of a mixture of carbon and lime is still below 80, measured by the test referred to, so that a carburizer made from carbon and lime alone would be commercially unsatisfactory.

The carburizing activity of mixtures of carbon and alkaline energizers will vary with the type of carbon, the method of compounding, and the percentage of energizer. It is not possible, therefore, to make a graph showing the absolute energizing power of these energizers for all carbons and proportions of carbon to energizer. However, with variations in the type and proportions of materials the general relationships expressed in Fig. 1 would not be disturbed even though the actual energizing powers of the individual materials might vary somewhat from the values shown.

The activities of carburizing compounds may be comparatively related to one another by a simple test in which cleaned test pieces of a suit-

able steel and of convenient size are weighed upon a chemical balance and then packed with carburizing compound in nickel-chromium alloy pots provided with fitted covers which are luted in place. The containers are then heated in a furnace, such as a gas-fired semimuffle furnace, to 1700° F. After a suitable period of time, say five hours, the containers are removed and cooled. The test pieces are then removed, cleaned if necessary, and again weighed. The gain in weight is a measure of the activity of the compound. Extensive experience with this method of testing relative carburizing activities has shown that case depth and degree of surface carburization closely parallel the gain in weight, for which reason this method may be taken as a standard for the purpose of obtaining relative carburizing efficiencies. A suitable test material is cold-rolled SAE 1020 steel cut into pieces 2½ inches long, 1 inch wide, and 1/8 inch thick, such specimens weighing approximately 63 grams. The pots used may suitably be about 7 inches deep and 2 inches inside diameter.

In applying such a test it is necessary to adopt some standard compound with which to make comparisons. The standard chosen in making the tests referred to herein was a commercially successful compound in pelleted form and consisting of 100 parts of carbon, 24 parts of barium carbonate, and 8 parts of lime, the three constituents being uniformly and intimately distributed through the mass of each pellet. The activity of this standard compound, measured by the gain in weight of a piece of SAE 1020 steel treated as just described, is arbitrarily given a test value of 100, and the activity of any other compound in the same heat may be figured as the relative gain in weight of its test piece. Thus, if a test piece treated with the standard compound gains 240 milligrams in weight, and a similar test piece in a second compound gains 200 milligrams in weight, the activity of the latter will be 200/240 of 100, or 83, which represents its relative carburizing activity.

It should be understood that the particular compound chosen as a standard is one having an average commercially acceptable activity. Other commercial compounds may have an activity, measured in the manner described, of 110 or 115, and some may have an activity of less than 100, say 90. Any compound having an activity of 80 or less measured in this manner would have no commercial value, and activities in excess of about 120 are meaningless because steels are not capable of absorbing carbon at a rate faster than that represented by an activity of about 115 to 120.

It has been proposed to add to ordinary carburizing compounds containing barium carbonate as the chief energizer, oxides of aluminum, nickel, lead, copper, manganese, iron, and other metals. Tests which I have made of such compositions show clearly that the additions proposed are not materially beneficial, and may be detrimental to the carburizers customarily used in the art and energized principally with barium carbonate, with sometimes sodium carbonate also, and that this is true whether or not lime be additionally present.

I have discovered, and it is upon this that my invention is predicated, that compositions consisting of carbon and lime may be activated to commercially acceptable activity by the addition of a heavy metal oxide, i. e., by such oxide these commercially unacceptable lime-carbon compositions become carburizers of satisfactory com-

mercial activity and of at least as great efficiency as the carburizers activated by barium or sodium carbonates, or both, now in commercial use. Furthermore, this activating effect of heavy metal oxide on carbon-lime compositions is specific to lime alone. In other words, the heavy metal oxide does not appear to super-activate energizers of the alkali and alkaline-earth groups other than lime.

Stated in other words, I have found that heavy metal oxides are capable of increasing the energizing power of lime on carbon to an extent such that a carburizer embodying characteristics rendering it entirely satisfactory from all commercial standpoints may be made from lime as the predominant or sole energizer through the use of such heavy metal oxide, and also that not only do the heavy metal oxides lack this beneficial effect upon the other energizers but may indeed decrease their energizing effect. Thus the essence of the invention resides in a carburizing compound in which lime and heavy metal oxide constitute the principal and commercially effective aids to carburization.

The term "heavy metal oxide" as used herein has reference to the oxides of nickel, iron, and chromium, and to a lesser extent manganese, although other heavy metal oxides may be used, such as those of cobalt and vanadium, all of which metals have atomic weights between 50 and 60. Because iron oxide is the commonest and cheapest of these oxides, and because for all practical purposes it is entirely satisfactory from the standpoint of its activating effect, reference will hereinafter be made to this member of this group by way of example, and not of limitation, in further illustration of the invention.

The relationship just expressed may be understood readily from a consideration of Fig. 3. The various graphs of this figure represent the carburizing activity of compounds made from carbon and 5 per cent of the particular carbonate indicated for each graph, plus iron oxide in the amounts which the abscissae of Fig. 3 represent. The composition made from carbon and lime alone showed a carburizing activity of less than 50. Such a carburizer would be totally inadequate for commercial purposes, modern commercial requirements demanding a carburizer having an activity of at least 80 as determined by the test referred to herein in all comparisons of such activity. But the addition of iron oxide to that carburizer in accordance with the invention progressively and substantially increased the activity so that at a content of slightly more than 1 per cent of iron oxide the compound reached commercially acceptable activity, and the activity was increased to substantially beyond the minimum commercially acceptable value by further additions of iron oxide.

In contrast, the other compounds, such as those of carbon and lithium carbonate, carbon and sodium carbonate, carbon and barium carbonate, and the others, some of which initially possessed high carburizing activity, were in each case detrimentally affected by the addition of iron oxide, thus proving that the use of heavy metal oxide is specific to lime alone of the energizers of the alkali and alkaline-earth metals.

As noted hereinabove, this was not to be expected because previous knowledge in the art, as represented, for example, by Figs. 1 and 2, indicated no abnormal characteristic for lime, and it was not to be expected that lime alone of the

seven common energizers would be thus responsive to heavy metal oxide.

I have found that relatively small amounts of lime and heavy metal oxide suffice to produce compounds of high and commercially acceptable activity, an advantage which reflects itself directly in low cost of the carburizing compound. For example, as little as 3 parts of lime, calculated as calcium hydroxide, will produce a fairly active compound when mixed with 100 parts of carbon and 3 parts of iron oxide. As indicated by Fig. 2, the energizing effect increases progressively with increase of lime, but too much lime will make the resultant compound mechanically weak with consequent shortening of its useful life, and ordinarily there is no advantage in using lime in excess of about 10 per cent. Likewise, as Fig. 3 indicates, substantial activation is effected by 1 per cent or less iron oxide, while for practical purposes the maximum effect appears to be reached at about 6 per cent.

For most purposes I now prefer to use from about 3 to 6 per cent of lime with about 2 to about 5 or 6 percent of iron oxide, and for most purposes an entirely satisfactory compound can be made from 5 parts each of lime and iron oxide with 100 parts of carbon. It will be understood that the use of other heavy metal oxides may require some change in relative proportions but that these changes can be determined readily by means known to those familiar with the art.

As is customary in the art, the carbon used in making the compounds may be derived from a variety of sources. I have discovered, however, that where coal is used as the source of carbon, it should be mixed with the lime and iron oxide prior to coking, at least where particularly high carburizing activity is desired. If coking coal is used, no other binder may be necessary, but since a major aspect of the invention resides in bonded compounds, as will appear, it will be understood that bonding may be achieved in other ways known to the art, such as by the use of molasses, for example.

The invention may be described further with reference to exemplary compositions.

*Example 1.*—100 parts by weight of powdered carbon, such as charcoal dust or pitch coke dust, are mixed with 5 parts of hydrated lime and 5 parts of finely powdered iron oxide. The mixture is then molded into pellets about  $\frac{3}{8}$  inch in diameter, using molasses as a binding agent. The pellets may be dried or heated to char the molasses binder.

*Example 2.*—As another example, 100 parts by weight of powdered low-ash coal are mixed with 5 parts of hydrated lime and 5 parts of iron oxide, and the mixture is then coked in containers out of contact with air. The resultant compound coke is crushed and screened to provide fragments of desired size, say those passing a 2-mesh and retained by a 4-mesh screen.

In the foregoing examples the base of the compound is a mixture consisting of 100 parts of carbon and 5 parts of lime. Such mixtures are scarcely more active than carbon alone in carburizing steel, and they have no possible commercial value. The surprising feature of the invention is, therefore, that the use of iron oxide increases the activity of such a composition to or beyond that of the usual commercial carburizing compounds containing large quantities of mixed and powerful energizers, and in which barium carbonate is chiefly relied on to produce the desired carburizing activity.

As further illustrative of the invention, reference will now be made to tests of various compounds which illustrate the principle on which the invention is predicated. These compounds were made according to the procedure of Example 2, and the compounds were tested in the manner just described. The following tabulation represents the constituents used in making the individual compounds and the average activity of each composition as determined from several successive heats. Although reference is made to coal in the tabulation it will be understood that this is to give the initial composition of the mixture, and that all of the mixtures were coked to prepare the compounds for testing.

| Compound | Composition                                 | Activity |
|----------|---------------------------------------------|----------|
| A        | Coal only.                                  | 35       |
| B        | 100 coal, 5 iron oxide.                     | 37 20    |
| C        | 100 coal, 5 calcium hydrate.                | 47       |
| D        | 100 coal, 20 calcium hydrate.               | 70       |
| E        | 100 coal, 5 calcium hydrate, 5 iron oxide.  | 115      |
| F        | 100 coal, 5 barium carbonate.               | 75       |
| G        | 100 coal, 20 barium carbonate.              | 110      |
| H        | 100 coal, 5 barium carbonate, 5 iron oxide. | 68 25    |

In considering the foregoing data it should be borne in mind that an activity of 100 represents approximately the average activity of the usual commercial carburizing compound, that an activity of 80 represents the lower limit which is commercially acceptable, and that an activity of 120 represents approximately the upper limit of useful activity as controlled by the ability of the steel to itself absorb carbon.

Compound A shows that carbon alone is a wholly ineffective carburizing material, and Compound B that iron oxide is virtually without effect in energizing coal. Compounds C and D show that lime alone, even in an amount of 20 per cent, does not alone render carbon active enough to be commercially acceptable. Compound E, however, shows that a composition made up in accordance with this invention possesses an activity vastly superior to that of carbon alone, carbon and iron oxide, or carbon and lime. Compound E is also superior to those made from barium carbonate (F, G), and Compound H shows how heavy metal oxide represses the powerful energizing effect of barium carbonate.

Comparison of Compound E with Compounds B and C shows further that the activity flowing from conjoint use of lime and iron oxide is more than merely additive. Thus, iron oxide alone (Compound B) increases the activity of coal alone (Compound A) but 2 points, and lime alone (Compound C) increases it only 12 points. Hence the use of 5 parts each of iron oxide and lime would increase the activity of Compound A (coal alone) 14 points if their joint use were merely additive. Actually, the activity of Compound E is 115, which is 80 points in excess of the sum of the activity of Compound A and 66 points more than the sum of the increases obtained with the constituents used singly in the same amounts.

These data are accordingly corroborative of Fig. 3, itself based on actual experimental data.

Some oxides exert a harmful effect upon these carburizers, and among these the oxides of silicon and lead are especially harmful, silica tending to reduce the activity of the compound when used for successive heats, and lead oxide tending to render the compound initially of low and unsatis-

factory activity. I have found that in the practice of the invention the iron oxide should be, accordingly, of rather high purity. For instance, iron oxides of high silica content show virtually no activating effect when used in the practice of the invention. On the other hand, iron oxides containing 98 per cent to 99 per cent of iron oxide are fully satisfactory. The same observations apply also to the other heavy metal oxides contemplated by the invention, i. e., they should be low in or free from impurities which would tend to repress the activating influence of the heavy metal oxide, and of these silicates, particularly aluminum silicates, are especially objectionable.

The purer iron oxides of commerce, such as those produced by precipitation from solution, by calcination of iron sulfate, and by oxidation of iron in contact with water, are sufficiently active for the purposes of this invention. I have found that the scale which is dislodged in the working, e. g., forging and rolling, of steel ingots, billets and the like, commonly known as "mill scale," affords a cheap source of iron oxide which is eminently satisfactory for the purposes of the present invention. This mill scale is friable and may be easily powdered with no tendency to pack or agglomerate during pulverization. When finely powdered it is a very heavy black material which is as effective for the purposes of the invention as the bulkier and more expensive iron oxides produced by precipitation or calcination methods to which reference has just been made. Also, the density of mill scale is advantageous because the dense powdered mill scale shows a lessened tendency to make soft coke or briquettes upon the heating of a mixture of it with lime and coal or other types of carbon.

In general, the ingredients, especially the heavy metal oxide, should be in finely powdered form, the coarser oxides being of slight benefit. Furthermore, the finely powdered oxide, lime and carbon should be intimately and uniformly mixed. Heavy metal oxide in the form of coarse particles, or unmixed with the carbon and lime, for instance when applied as a separate layer to the surface of the compound, does not afford the substantial benefits of this invention.

To this end the mill scale, or other heavy metal oxide, should be finely powdered. For instance, it may be ground so that 98 per cent or 99 per cent of the material will pass a 200-mesh standard screen.

To insure intimacy of their mixing the ingredients may be mixed in a ball mill. The mixture may be coked, or it may be formed into pellets which are then coked. It will be evident that an intimate, bonded mixture of the powdered ingredients may be produced upon the surface of supporting pellets or fragments, whether this base support be active or inactive. Most suitably, however, the materials are reduced to finely powdered form, mixed and then bonded by any suitable procedure.

A feature of eminent importance in achieving the highest activity in the practice of the invention is that the compositions should be subjected to a bonding treatment, in the course of production of the compound. Bonding is desirable, of course, to maintain intimacy, uniformity and positive contact, and to avoid separation and segregation of the ingredients of the composition in handling and using it. I have found, however, that even where segregation is avoided without bonding it is still advantageous to bond the ingre-

dients firmly together if the full advantage of the invention is to be attained. Moreover, this feature appears to be of greater importance in the practice of this invention than in the case of the usual carburizers energized chiefly with barium carbonate. As evidencing this reference is made to the following tests.

*Example 3.*—100 parts by weight of powdered low-ash coking coal were mixed intimately with 5 parts of powdered hydrated lime and 5 parts of finely powdered mill scale. The mixture was coked and then crushed to a fine powder.

*Example 4.*—Some of the coal used in Example 3 was coked, crushed to a fine powder, and 100 parts of this powdered coke then mixed with 8 parts of finely powdered mill scale and 8 parts of lime. The reason for increasing the amount of lime and mill scale in this composition was that the particular coal used contained about 37 per cent of matter volatile in coking at 1700° F. Allowance was made therefore for the evolution of that volatile matter in the coking of the coal used in this example so that the compositions of Examples 3 and 4 finally consisted of the same proportions of identical constituents, each in a fine state of sub-division, the difference being that in the process of manufacture one (Example 3) had been bonded and the other (Example 4) had not.

Carburizing tests upon these compositions showed an activity of 117 for the bonded mixture of Example 3, and of 75 for the mixture of Example 4 which had not been bonded. After using the compositions for several heats, the unbonded mixture of Example 4 was made into pellets, using molasses as a binding agent, and it then showed an activity of 120, as contrasted with 75 in the unbonded condition, thus bringing it to the activity of Example 3 and further evidencing the value of bonding.

*Example 5.*—In another series of tests 100 parts by weight of finely powdered pitch coke containing approximately 1/2 per cent of ash and 9 per cent of volatile matter was mixed with 4 parts of powdered iron oxide and 8 parts of hydrated lime. Part of this mixture (Ex. 5-A) was retained in the dry mixed condition, and part was mixed with about 20 per cent of tar to make a satisfactory bond when the mixture was briquetted and coked. This coked mixture was then crushed to a fine powder (Ex. 5-B). Carburizing tests showed an activity of 115 for the material (Ex. 5-B) that had been bonded and then powdered, and 80 for the loose mixture (Ex. 5-A).

As coking coal is a cheap and readily available source of carbon, and offers, moreover, in coking the advantage of a binding means, it would be a desirable material to use in the practice of this invention. Coal, moreover, has been found satisfactory for the manufacture of ordinary carburizing compounds energized chiefly with barium and sodium carbonates.

Such coals, however, may not produce satisfactory carburizing compound in accordance with this invention, apparently because, as mentioned hereinabove, the carburizers provided by the invention are peculiarly sensitive to the poisoning effects of silicon oxides and other oxides and oxidic materials such as alumina and silicates, especially aluminum silicate, which is the chief ingredient of coal ash. I have found, however, that by the use of coking coal containing less than 4 per cent of ash, and most suitably less than 2 per cent of ash, the benefits of the invention are fully realized. Thus, excellent and inexpensive carburizing compound can be made by mixing 100

parts of finely powdered coking coal containing less than 4 per cent of ash with small amounts of lime and heavy metal oxide, say 5 parts each of lime and mill scale, coking the mixture and crushing the compound coke to secure fragments of desired sizes.

As indicative of the influence of coal ash upon the carburizers provided by this invention, compounds made by coking briquetted pellets about 10  $\frac{3}{8}$  inch in size made from a mixture of floated Eastern Kentucky coal containing 1.2 per cent of ash, with 5 parts each of lime and mill scale showed an initial activity of about 120 which was sustained unusually well in re-use. Compounds 15 made in the same manner and using the same proportions, but made from Eastern Kentucky coal with 5 per cent of ash, Pittsburgh seam coal with 7 per cent of ash, and Cambria County (Pennsylvania) coal with 4.5 per cent of white 20 ash, showed but about 80 per cent activity, and the activity lessened rapidly with re-use.

While the preferred embodiment of the invention contemplates compounds consisting of carbon, lime and heavy metal oxide, it will be appreciated that other substances may be added for 25 special purposes, including amounts of other energizers, as long as the activity characteristic of the invention is not adversely affected. However, the simple compositions stated give fully satisfactory 30 carburizing activity, even to that which supplies carbon at the maximum rate at which it can be absorbed by steel, and therefore they are most desirable for most purposes.

From what has been said many of the advantages 35 of the carburizing compounds made by adding iron oxide or other heavy metal oxide to a mixture of carbon and a small amount of lime as the dominant and commercially effective or only energizer will be understood by those skilled in 40 the art. These compounds are characterized by high activity at all the usual carburizing temperatures, and they exhibit unusually well-sustained activity when the compound is subjected to repeated heats. For instance, compounds made as 45 described herein have been maintained at their original high activity by adding to the used compound after each heat only 5 to 10 per cent of fresh compound, whereas it is customary and necessary to add 10 to 35 per cent of fresh compound of the older commercial types.

A major advantage is the low cost due to the use of small amounts of inexpensive calcium 50 hydrate and iron oxide instead of rather large amounts of the more expensive barium carbonate. The actual saving may amount to nearly 10 per 55 cent of the selling price of the usual compounds energized chiefly with barium carbonate.

Of especial interest to the user of carburizing compound is the fact that compounds according 60 to this invention produce unusually smooth and evenly carburized surfaces. The compounds heretofore used commercially containing barium carbonate or sodium carbonate, or both, frequently produces rough spots and small semi-soluble 65 adhesions upon the steel surfaces, and the areas under these adhesions may be insufficiently carburized to harden successfully, giving rise to "soft spots" on the steel and the necessity of either re-carburizing or discarding the parts so affected. The surface of steel carburized with the compounds in accordance with this invention has a 70 smooth gray appearance with no sign of roughness or adhesions and is evenly carburized over the entire area exposed to the compound, i. e., the 75 rough spots encountered in the use of the prior art

carburizers are avoided through the practice of this invention.

When a carburizing pot containing the usual barium carbonate product is opened, especially if it be opened while still hot, the dust created is found to be particularly offensive to the sense of smell and irritating to the respiratory tract. In contrast, the dust and odor (if any) arising from compound made from carbon, lime and iron oxide in accordance with this invention is not offensive 10 or irritating. Also, barium carbonate energized compound may be objectionable because barium compounds are known to be poisonous, which is not true of lime.

It is well known that carburizing compounds 15 containing sodium carbonate, or sodium and barium carbonates, attack alloy carburizing pots, in some instances quite rapidly, causing corrosion and the formation of the so-called "cancers," which materially shorten their useful life. While 20 barium carbonate alone does not attack the pots so rapidly, it is not certain that considerable, if slow, attack and injury do not, nevertheless, occur. In extensive and prolonged observation and 25 test upon the compounds provided by this invention I have not detected any observable sign of attack upon the alloy containers in which it was packed. It appears, therefore, based partly upon this observation and partly upon the unusually clean surface of the steel packed in my new compound, that its use will lengthen the usual life of 30 these alloy carburizing pots, thus further increasing carburizing economies.

In summary, earlier investigators have, as previously stated, sought to provide carburizers of 35 increased activity by adding metal oxides to carburizing mixtures initially having a commercially acceptable activity attained by the use of large amounts of energizers, chiefly barium. The addition of metal oxides to these highly active mixtures can evidently improve them little, if at all, 40 because of the inability of the steel itself to absorb carbon faster than supplied by such a compound energized principally by barium carbonate and not containing the ancillary metal oxide. Furthermore, as shown by Fig. 3, any activation of 45 calcium energizer present in the mixture would be offset by the adverse effect of the metal oxide on the barium and other energizers, and this probably explains why these prior proposals have 50 been without beneficial result. Tests upon these particular mixtures have fully confirmed these 55 statements.

It should be understood that the belief is that the so-called energizers, such as barium carbonate and calcium hydroxide, are not effective as 55 energizers until they have been reduced to the corresponding oxides, the reduction occurring 60 ordinarily when the compound is raised to carburizing temperatures. Likewise, I now believe 65 that the iron oxide and the like, which serve to increase the energizing effect of calcium oxide in accordance with this invention, are not effective until they have been reduced to finely divided metal, as iron or nickel, this reduction, also, occurring when the compound is heated 70 to carburizing temperatures. For this reason it is possible to substitute finely divided metals of this sort for the heavy metal oxides or other reducible compounds, although probably that 75 would not be economical since the oxide affords a cheaper source of the metal. In this connection it is interesting to observe that the molecular weight of the calcium oxide and the atomic weight of those metals which increase its ef-

fectiveness, as well as the atomic weight of the metal being carburized, all fall within a short range of each other, being grouped about the number fifty-five.

5 Also, while reference has been made in the claims to "lime" it will be understood that this contemplates not only the oxide of calcium, but also its carbonate, hydroxide, or other calcium compound reducible to the oxide, all of which 10 may be used.

Most of the claims appended to this specification have been written in the usual way, i. e., by expressing contents of carbon or carbonaceous material and energizer, etc. Most carbonaceous 15 materials evolve gases and lose weight in being heated, and this loss of weight may be large; for instance, the usual commercial charcoal will lose 25 per cent to 30 percent of its weight in being heated to carburizing temperatures; bituminous 20 coal may lose 15 per cent to 40 per cent; sawdust, tan bark and the like may lose as much as 85 per cent. Likewise, weight changes are involved in converting energizing carbonate to oxide, and heavy metal oxide to metal. For these reasons 25 some claims are based upon the composition of the compounds at operating temperature, say about 1700° F., since this gives a comparable relation of the constituents in actual use.

According to the provisions of the patent statutes, I have explained the principle and manner 30 of practicing my invention and have illustrated and described what I now consider to represent its best embodiment. However, I desire to have it understood that, within the scope of the appended claims, the invention may be practiced 35 otherwise than as specifically illustrated and described.

I claim:

1. A carburizing compound comprising carbonaceous material, lime as the principal effective added energizer, and an activity-promoting material selected from the group consisting of finely divided metal having an atomic weight 40

between 50 and 60 and finely divided reducible compound of such metal, said activity-promoting material being present in an amount sufficient to render the compound of commercially acceptable carburizing activity.

2. A carburizing compound comprising a bonded mixture of carbonaceous material, lime as the principal effective added energizer, and an activity-promoting material selected from the group consisting of finely divided iron and iron oxide in an amount sufficient to render the compound of commercially acceptable carburizing activity.

3. A carburizing compound comprising a bonded mixture of carbonaceous material, at least about 3 per cent of lime as the principal effective added energizer, and at least about 2 per cent of finely divided oxide of a metal having an atomic weight between 50 and 60 which cooperates with said lime to render the compound 20 of commercially acceptable carburizing activity.

4. A carburizing compound comprising a bonded mixture of carbonaceous material, at least about 3 per cent of lime as the sole added energizer, and at least about 2 per cent of iron 25 oxide, said lime and iron oxide cooperating to render the compound of commercially acceptable carburizing activity.

5. A carburizing compound comprising a bonded mixture of carbonaceous material, about 30 5 per cent of lime as the sole added energizer, and about 5 per cent of finely divided iron oxide, said lime and iron oxide cooperating to render the compound of commercially acceptable carburizing activity.

6. A carburizing compound comprising a bonded mixture of carbonaceous material, lime as the principal effective added energizer, and an amount of finely divided metal having an atomic weight between 50 and 60 sufficient to render the compound of commercially acceptable carburizing activity.

HUGH RODMAN.